

965,050.

J. O. E. TROTZ.  
PROCESS OF ROLLING INGOTS.  
APPLICATION FILED OCT. 6, 1908.

Patented July 19, 1910.

2 SHEETS—SHEET 1.

Fig. 1.



Fig. 2.



Witnesses

Roy J. Tolman.  
Penelope Cumberback

Inventor

Johan D. E. Trotz.  
By Henry Wood Fowler  
Attorney

J. O. E. TROTZ.  
PROCESS OF ROLLING INGOTS.  
APPLICATION FILED OCT. 6, 1908.

965,050.

Patented July 19, 1910.

2 SHEETS—SHEET 2.

Fig. 3.



Fig. 4.



## *Witnesses*

Roy D. Tolman.  
Penelope Comberbach

Inventor  
Johan O.E. Trotz.  
By Henry Wood Fowler  
Attorney

# UNITED STATES PATENT OFFICE.

JOHAN O. EMANUEL TROTZ, OF WORCESTER, MASSACHUSETTS.

## PROCESS OF ROLLING INGOTS.

965,050.

Specification of Letters Patent. Patented July 19, 1910.

Application filed October 6, 1908. Serial No. 456,461.

*To all whom it may concern:*

Be it known that I, JOHAN O. EMANUEL TROTZ, a citizen of Sweden, residing at Worcester, in the county of Worcester and 5 Commonwealth of Massachusetts, have invented a new and useful Improvement in a Process of Rolling Ingots, of which the following is a specification, accompanied by drawings, forming a part of the same, in 10 which—

Figure 1 is a plan view of a three high rolling mill. Fig. 2 is a diagrammatic view of the rolls, showing the series of passes arranged for my improved process. Figs. 3 15 and 4 are vertical sectional views.

Similar reference characters refer to similar parts in the different views.

My present invention relates to a new and improved method of rolling ingots, and to 20 a three high rolling mill for carrying my invention into effect whereby the number of consecutive passes required for a given reduction of the ingot is reduced in number, enabling the length of the rolls to be materially decreased, thereby securing greater 25 rigidity in the rolls and greater accuracy in the dimension of the rolled metal.

In carrying my present invention into practice I employ a three high mill having 30 a series of consecutive passes for the reduction of the ingot arranged in upper and lower rows, and having means for raising and lowering the ingot from the plane of one row to that of the other, as is common 35 in three high mills.

It has been the practice heretofore to reduce the ingot in cross section in one dimension only by the first pair of upper and lower passes, and subsequently reduce the 40 ingot in cross section in the other dimension by the next succeeding pair of upper and lower passes, turning the ingot between each subsequent pair of passes.

By the practiced method of rolling ingots 45 in a three high mill, as above described, the height of the first pass in the second pair of passes and in each subsequent pair of passes is sufficiently less than the width of the last pass in the preceding pair of passes to give 50 the desired reduction of the ingot, but is greater than the height of the preceding pass.

In a three high mill adapted to carry my

present process into practice the height of the first pass in the second pair of passes 55 and each subsequent pair of passes is less than the height of the last pass in the next preceding pair of passes. By the method as now practiced the ingot is reduced in one dimension only by each pair of passes, requiring a second pair of passes for its reduction in the other dimension, and necessitating rolls of considerable length for the requisite reduction of the ingot.

By my process as hereinafter described, I 65 make each pair of passes in the rolls do double duty. The number of passes in each set of rolls in a three high mill can be reduced in number, thereby shortening the rolls and rendering them more stiff and 70 rigid. I have found in practice that by my improved process the rolls of a three high mill can be reduced by my improved method of rolling approximately one third in length, giving rolls of sufficient rigidity and 75 stiffness to enable the ingot to be rolled to its finished size with sufficient exactness, by means of a finishing pass at the extreme end of the rolls and next the roll housings.

Referring to the accompanying drawings, 80 which represent a three high rolling mill having its passes constructed and arranged in accordance with my new and improved method of rolling ingots, A represents the roll housings and C, D and E the rolls of a 85 three high mill journaled therein. Between the lower and middle rolls C and D are the reducing passes F, G, H and I, and between the middle and upper rolls D and E are the reducing passes J, K, L and M, and between 90 the lower and middle rolls C and D is a final or finishing pass N. Upon opposite sides of the rolls are ingot supporting tables O and P, capable of being raised and lowered by hydraulic plungers or other means in position to support the ingots in alinement with either the lower or upper row of passes between the rolls C, D and E.

In the drawings the tables O and P are represented by solid lines in position to support the ingot in alinement with the lower row of passes, and by the broken lines O' and P' in position to support the ingot in alinement with the upper row of passes.

The ingot Q is first rolled through the 105 pass F, Fig. 2, and returned through the

pass J, the movement of the ingot being indicated by the arrows *a* and *b*. The width of the first pair of passes F and J is substantially the width of the ingot, but the height of the first pass F is sufficiently less than the vertical thickness of the ingot to effect the desired reduction. The width of the second pass J is the same as the pass F, but its vertical height is sufficiently less than the vertical height of the first pass F to accomplish the second reduction in the thickness of the ingot.

In the present instance the ingot Q, having its cross section indicated by the broken lines  $Q^1$  and approximately 12" square, in passing through the pass F into the position indicated at  $Q^2$  is reduced in thickness to 9 $\frac{1}{2}$ ", having its cross section indicated by the broken lines  $Q^3$ . The tables O and P are then raised into alignment with the upper row of passes and the ingot brought into the position at  $Q^4$ , to be returned through the upper pass J into the position at  $Q^5$ , and having its thickness still further reduced to 8" as indicated in cross section by the broken lines  $Q^6$ . The tables O and P are then lowered into the position shown by solid lines in Fig. 4 and the ingot is turned one quarter revolution around its longitudinal axis, so as to be supported on its edge as shown at  $Q^7$ , the dimensions of the ingot in cross section being indicated at  $Q^8$ , having a horizontal width of 8" and a vertical thickness of say 12". The ingot is then returned in the direction of the arrow *c* through the first pass F into the position at  $Q^9$ , with its cross section reduced in thickness to 9 $\frac{1}{2}$ ", as indicated by the broken lines  $Q^{10}$ . The tables are then raised bringing the ingot into the position at  $Q^{11}$ , from which it is returned in the direction of the arrow *d* through the pass J into the position indicated at  $Q^{12}$ , having its vertical thickness reduced to 8".

The width of the second pair of passes G and K is equal to the height of the last pass J in the first pair of passes, in the present instance 8", while the height of the first pass G of the second pair is sufficiently less than the height of the last pass of the preceding pair to accomplish the desired reduction in the thickness of the ingot which, in the present instance, is 6 $\frac{3}{4}$ ". The ingot after having been returned for the second time through the pass J, as above described, and having its cross section reduced to 8" in thickness and to 8" in width plus a slight increase, due to the spreading of the ingot during its two last reductions, is then turned one quarter revolution so as to be supported upon one of its 8" sides, and is then rolled through the pass G, leaving its dimensions 8" wide by 6 $\frac{3}{4}$ " in thickness. The ingot is then returned through the upper pass K of the second pair by which its thickness is still

further reduced, in the present instance, to 65 5 $\frac{1}{2}$ ". The ingot is then turned one quarter revolution and rerolled through the passes G and K, reducing the ingot in cross section to approximately 5 $\frac{1}{2}$ " square.

The third pair of passes H and L have 70 their width equal to the height of the last pass in the preceding pair which, in the present instance, is 5 $\frac{1}{2}$ ", but the height of the first pass H is less than the height of the last pass in the preceding pair, in the 75 present instance, 5", while the height of the second pass L in the pair is 4". The ingot is then rolled twice through the third pair of passes H and L, with one quarter turn between each rolling as previously described, 80 and the same method is pursued with regard to the fourth pair of passes I and M. After the final rolling through the pass M the ingot is rolled through the finishing pass N, which leaves the rolled metal the exact dimensions required in cross section.

By the above method of rolling, the number of passes in the rolls and, consequently, the length of the rolls is considerably reduced from that required in the method now 90 commonly practiced. I have found, for example, that the rolls of a three high mill when made in accordance with the method now commonly practiced are over 80" in length, whereas the same reduction in the 95 ingot can be accomplished by my improved method of rolling with rolls 53" in length. This reduction in the length of the rolls and reduction in the number of passes not only reduces the cost of the rolls, but also increases their stiffness and rigidity as the distance between the housings is reduced.

I claim:

1. The method of rolling ingots, comprising reducing the ingot in cross section in 105 one dimension by rolling it through a pass of the desired dimension, turning the ingot a quarter turn around its longitudinal axis and rolling it through the same pass in the opposite direction to accomplish its reduction in the other dimension.

2. The method of rolling ingots, comprising rolling the ingot through each pass in opposite directions and imparting a quarter turn around its longitudinal axis to the ingot between its passages through the pass in said opposite directions, whereby said ingot is reduced in two dimensions by said rolling in each pass.

3. The method of rolling ingots, comprising rolling the ingot twice through each pass and imparting a quarter turn to the ingot around its longitudinal axis between each rolling through each pass.

4. The method of rolling ingots, comprising reducing the cross section of the ingot in one dimension by rolling it through a pass of the desired dimension, turning the ingot

a quarter turn around its longitudinal axis and reducing it in cross section in the other dimension by the same pass.

5. The method of rolling ingots in a mill having a series of passes, comprising reducing the ingot in cross section in two dimensions by each pass in said series, turning the

ingot a quarter turn around its longitudinal axis between such reduction by each pass and transferring the ingot to the succeeding pass. 10

JOHAN O. EMANUEL TROTZ.

Witnesses:

PENELOPE COMBERBACH,  
RUFUS B. FOWLER.